

## UNITED STATES PATENT OFFICE

2,194,932

## TREATMENT OF TEXTILE MATERIAL

Charles N. Frey, New York, N. Y., and Stephen Jozsa, Chicago, Ill., assignors to Standard Brands Incorporated, New York, N. Y., a corporation of Delaware

No Drawing. Application July 9, 1936,  
Serial No. 89,848

11 Claims. (Cl. 195—64)

The invention relates to a process for desizing and increasing the wettability of textile material and to a composition therefor. More particularly, it relates to a procedure for desizing cotton and 5 mixed goods while simultaneously improving the wettability thereof and includes correlated improvements and discoveries whereby these desired results are obtained.

When preparing textiles for the dye bath, it 10 has been the usual practice that they were first placed in a hot dilute solution containing an active starch liquefying enzyme, such as diastase. The excess of solution was removed usually by 15 passing them through wringer rolls, and they were then maintained in a heated condition for a period of time so that the starch carried by the textile material was digested preferably substantially completely following which the material was rinsed and dried. It was found that materials 20 so treated were deficient with respect to wettability; that is, when they were introduced into the dye bath the dye solution did not immediately enter the material which was rather more or less repellent. This resulted in an uneven and spotted dyeing of the so treated materials.

It is an object of the invention to provide a 25 procedure whereby textile materials may be desized and have their wettability increased in a simple, single treating procedure with a result that subsequent dyeings may be made uniformly and without spotting.

Another object of the invention is to provide a 30 procedure for the treatment of textile materials in which such materials are placed in a bath containing a starch liquefying enzyme and a phosphatide, e. g., lecithin, and which may be readily, effectively and economically carried out in commercial practice.

A further object of the invention is to provide 35 a bath for simultaneously desizing and increasing the wettability of textile materials which contains a diastatic enzyme and lecithin.

A specific object of the invention is the provision 40 of a composition for utilization in the treatment of textile materials containing a diastatic enzyme of about 300° Lintner value and from 1 to 4% of lecithin.

Other objects of the invention will in part be 45 obvious and will in part appear hereinafter.

The invention accordingly comprises the several 50 steps and the relation of one or more of such steps with respect to each of the others, and the composition possessing the features, properties, and the relation of constituents, which are exem-

plified in the following detailed disclosure, and the scope of the invention will be indicated in the claims.

In the practice of the invention, textile material may be desized and the wettability increased 5 by treating with a composition, at a suitable temperature, containing an active starch liquefying enzyme, e. g., a diastatic enzyme containing solution, and a phosphatids. The phosphatide preferred is lecithin which may be the usual product of commerce as prepared from the soy bean.

It will be understood that reference herein to lecithin is with respect to that product which is ordinarily purveyed and that the utilization of a pure lecithin will entail a corresponding variation in the quantities given. As the source of an active liquefying enzyme there may be employed a solution of a diastatic enzyme having a Lintner value of about 300°.

The lecithin utilized may be admixed with 20 the diastase solution under energetic agitation, as with a high speed mixer, that is, one operating at from 10,000 to 15,000 R. P. M. Further, a rather concentrated solution of lecithin may be prepared and then this solution admixed with 25 the diastatic enzyme solution in suitable amounts.

Thus, a 1 to 5 solution or emulsion of lecithin may be made by gradually adding a small amount of warm (about 45° C.) water to lecithin and mixing. The addition of the lecithin to the diastatic enzyme solution may be in an amount of 30 0.5 to 4% and the admixture stored without material diminution of the liquefying power of the enzyme.

Treatment of textile material may be effected 35 by way of illustrative example in a bath containing about 1% of a diastatic enzyme solution having a Lintner value of 300° thus giving a treating bath having a Lintner value of about 3° and containing about 1% of lecithin. The textile material is immersed therein at a temperature of about 50° C. and allowed to remain for a period of twelve hours, suitably overnight. It is then withdrawn from the treating bath; the excess of bath liquid removed by suitable means, as passing between wringer rolls, and maintained at a temperature which may be 60 to 65° C. for a suitable time to permit digestion of starch carried by the material, after which it is rinsed and dried.

Textile material so treated has a markedly increased wettability and subsequent dyeings thereon may be made with uniformity and lack of spotting. The wettability of material thus treated was observed by recording the time required for a drop of water to penetrate entirely into the 50 55

material. The penetration of a check was found to require thirty-two seconds, whereas material treated in a bath to which a diastatic solution containing 0.5% of lecithin had been added gave

5 a penetration in twenty-two seconds, when 1% of lecithin was used the penetration was 8 seconds, 2%, six seconds, and 4%, five seconds. The corresponding amounts of lecithin contained in the bath on the basis of 0.5, 1, 2 and 4% content of the diastatic enzyme solution was 0.005, 0.01, 0.02, and 0.04 respectively.

While the manner in which the lecithin increases the wettability of the goods is not known, nevertheless, it appears to be that during the 15 digestion of the starch carried by the textile material through the action of diastatic enzymes the lecithin attaches itself to the surfaces of the fibers constituting the material and remains thereon during the subsequent rinsing and drying operations. Consequently, when the dried material is placed into a dye bath, the lecithin tends to spread the water of the dye solution quickly and thoroughly throughout the fibers thus yielding a uniform and even dyeing.

20 25 The textile material treated in accordance with the foregoing procedure is not only thoroughly desized, but possesses also a high degree of wettability so that when introduced into a dye bath there results an even dyeing and the rate at which the dye penetrates the fiber is increased. Furthermore, the material is without any undesirable feel or acrid odor.

Since certain changes in carrying out the above process, and certain modifications in the composition which embody the invention may be made without departing from its scope, it is intended that all matter contained in the above description shall be interpreted as illustrative and not in a limiting sense.

40 It is also to be understood that the following claims are intended to cover all of the generic and specific features of the invention herein described, and all statements of the scope of the invention which, as a matter of language, might be said to fall therebetween.

45 Having described our invention what we claim as new and desire to secure by Letters Patent is:

1. A process for desizing and increasing the wettability of textile material which comprises treating textile material with a composition containing an active starch liquefying enzyme and a phosphatide.

50 55 2. A process for desizing and increasing the wettability of textile material which comprises treating textile material in a bath containing an active starch liquefying enzyme and a lecithin.

3. A process for desizing and increasing the wettability of textile material which comprises treating textile material in a heated bath containing a diastatic enzyme and lecithin.

4. A process for desizing and increasing the 5 wettability of textile material which comprises preparing a bath containing a diastatic enzyme and lecithin, heating, immersing the textile material therein, withdrawing, maintaining in a heated condition until starch contained in said 10 textile material has undergone digestion, and then rinsing and drying.

5. A process for desizing and increasing the wettability of textile material which comprises preparing a bath containing a diastatic enzyme 15 and lecithin, heating at a temperature of about 50° C., immersing the textile material therein, withdrawing, maintaining in a heated condition until starch contained in said textile material has undergone digestion, and then rinsing and dry- 20 ing.

6. A process for desizing and increasing the wettability of textile material which comprises preparing a bath containing about 1% of a 300° Lintner diastatic enzyme composition and lecithin 25 in an amount of about 0.005 to 0.04%, heating to a temperature of about 50° C., immersing the textile material in said bath, withdrawing, removing excess liquid, maintaining in a heated condition until starch carried by said textile material 30 is substantially digested, and then rinsing and drying.

7. A composition of matter for the treatment of textile material which comprises in solution an active starch liquefying enzyme and a phosphatide.

8. A composition of matter for the treatment of textile material which comprises in solution a diastatic enzyme and lecithin.

9. A composition of matter for the treatment 40 of textile material which comprises a diastatic enzyme solution having a Lintner value of about 300° and containing 0.5 to 4% of lecithin.

10. A composition of matter for the treatment 45 of textile material which comprises a bath for desizing and increasing the wettability of textile material containing a diastatic enzyme, and lecithin in an amount of 0.005 to 0.04%.

11. A composition of matter for the treatment 50 of textile material which comprises a bath for desizing and increasing the wettability of textile material containing a diastatic enzyme, and lecithin in an amount of 0.005 to 0.04%, and having a Lintner value of about 3°.

CHARLES N. FREY. 55  
STEPHEN JOZSA.